

Jan. 11, 1972

HIDEO WATASE ET AL  
PROCESS FOR PREPARING FIBERS OF THE POLYESTER  
SERIES HAVING DIFFERENT DYEABILITY  
Filed Feb. 4, 1969

3,634,580

Fig. 1



Fig. 2



Fig. 3



Fig. 4



**1**

3,634,580

**PROCESS FOR PREPARING FIBERS OF THE POLYESTER SERIES HAVING DIFFERENT DYEABILITY**

Hideo Watase, Akira Kobayashi, Tadashi Hirakawa, and Atsushi Sugiyama, Tokyo, Japan, assignors to Teijin Limited, Osaka, Japan

Filed Feb. 4, 1969, Ser. No. 796,469

Claims priority, application Japan, Feb. 7, 1968,  
43/7,542

Int. Cl. B29c 25/00

U.S. Cl. 264—342

1 Claim

**ABSTRACT OF THE DISCLOSURE**

Process for preparing fibers of the polyester series having different dyeability, characterized by subjecting fibers of the polyester series to a non-contact heat treatment momentarily under very low tension in the atmosphere kept at a temperature above the melting point of said fibers, whereby remarkable different dyeability is imparted to the fibers along the fiber length direction.

The present invention relates to a process for preparing fibers of the polyester series having different dyeability. More particularly, the present invention relates to a process for preparing fibers of the polyester series having remarkable dyeing differences along a direction of length of the fibers. Heretofore, as a process for preparing fibers having varying shades of color brought about by dyeing, a process of unequal drawing after spinning has been known. Portions where a draw ratio is low are dyed in a deep color and portions where a draw ratio is high are dyed in a thin color. However, when it is attempted to obtain fibers having a large difference in shade, the tenacity of the fibers lowers. Namely, when a portion of a very low draw ratio, for instance, non-drawn portion is put aside and the remaining portion is drawn, the difference in shade becomes large; however, the mechanical properties of the fibers remarkably deteriorate. So far, fibers having practical mechanical properties and large difference in shade have not been obtained. Also by such a process it is difficult to obtain fibers having large difference in shade wherein color changing lengths are short; this becomes more difficult in fibers prepared continuously at a high speed.

The present invention improves said various deficiencies brought about in concomitance with imparting to fibers of the polyester series different dyeability through a mass production technique. An object thereof is to provide fibers of the polyester series having different dyeability so that when dyed the fibers show a remarkable difference in shade along a direction of length of the fibers, wherein mechanical properties of said fibers are retained on the level of practical use.

Another object of the present invention is to provide fibers of the polyester series wherein change in shade occur at short intervals, and the feel of the fiber is improved by development of peculiar crimps in said fibers of the polyester series having different dyeability.

A further object of the present invention provides a process for continuous mass production at a high speed of fibers of the polyester series having the aforementioned remarkable different dyeability as well as improved feel.

Brief explanation of the accompanying drawings is as follows.

FIG. 1 is an enlarged side elevation of filaments of the polyester series having non-periodic different dyeability provided by the process of the present invention. FIG. 2 is an enlarged view of said filaments of FIG. 1. FIG. 3 is a longitudinal sectional view of a heat treating apparatus

**2**

used in the present invention. FIG. 4 is a graph showing relation of heat treating temperature and dyeability of treated fibers.

It has been found that in order to obtain a sufficient deep color in polyester fibers, it is necessary that dyeability of the fibers as a whole be improved above a certain standard; moreover, said dyeability has a close relation to the degree of crystallinity of the fibers and it is necessary that the degree of crystallinity of the fibers after treatment be at least 40%. It has been found that when fibers of the polyester series are subjected to a momentary non-contact heat treatment under a very low tension in the atmosphere kept at a temperature above the melting point of the fibers, different dyeability is brought about in the direction of length of the fibers. At the same time, a special crimp is brought about in the fibers per se. With regard to the heating apparatus, the present invention carries out non-contact heating as shown in FIG. 3. In a cylinder 2 a high temperature atmosphere is created and fibers of the polyester series are made to pass therethrough under low tension. The passing time is momentary, e.g. 0.02–0.10 second. In FIG. 1, many filaments 1' gather and they are loosely intertwined in multi filamentary state. When said filaments are dyed after being subjected to the heat treatment of the present invention, difference in a shade of color is brought about on said filament. In FIG. 1 and FIG. 2 a is a deep color portion, while b is a thin color portion. Coloration of a shade of color is in many cases non-periodic. It is possible that when said filaments pass momentarily through a high temperature (above the melting point of the filaments) gas, perhaps the filaments are not melted but they receive sudden heating. That heating is unequal. For instance, when there is a stream in a heated gas, when the side surface of said filaments directly facing said stream is compared with the side surface of said filaments at the rear of said surface, there is a difference in heating. Between outer filaments and inner filaments constituting a filamentary yarn, there is naturally great difference in heating. Generally filaments shrink by heating. Said shrinkage varies in proportion to the temperature of heating. In case of filaments, a plurality of monofilaments shrink en masse, however, variation thereof becomes very complicated. When shrinkage is great, coloration becomes strong and in portions shrinking little, coloration becomes weak. As mentioned above, when fibers of the polyester series are momentarily heated at a temperature above the melting point of said fibers, fibers shrink and as a result shrunken parts are dyed deeply, which is shown in FIG. 4. Namely, FIG. 4 shows the relationship between the heat treating temperature (°C.) (abscissa) and the dyeability (ordinate) in case of heat treating polyethylene terephthalate filaments in high temperature air under low tension for 0.15 second as an example. The dyeability as herein referred to is determined as follows. Namely, the fibers are dyed in a boiling dye bath of Dispersal fast Scarlet B, 4% O.W.F. for 30 minutes, the fibers are dissolved in a solution of orthochlorophenol and the dyeability is determined from an optical density of 515 m $\mu$ , indicated by a relative value when the dyeability of the non-treated fibers is made 1. For the foregoing reasons different dyeability develops. Namely, due to sudden heating filaments shrink. Because the heating is unequal, there is unevenness in shrinking. Due to this unequal shrinking so-called different dyeability occurs, because portions shrinking much are dyed deeply and portions shrinking little are dyed weakly. Also in the present invention there is development of peculiar crimp, which is caused by shrinking of the filaments at the time of heat treatment.

Next, concerning different dyeability of fibers of the polyester series due to heat treatment, when the cause

therefor is considered and studied experimentally, it is found that in development of different dyeability various conditions participate. When illustrated, they are a high or low temperature, a long or short time of heat treatment and tensile strength imposed on the filaments. These various elements do not work alone but have intimate correlation. At first unequal shrinking of the filaments causing development of different dyeability is made one target and what roles these various elements play thereto will be considered.

As a temperature, a fluid temperature in the heat treating zone is considered, which temperature is above the melting point of fibers of the polyester series, preferably a temperature higher than said melting point by at least 100° C. is adopted. When the melting point is 270° C., the fluid temperature for heating is preferably at least 370° C. As the highest temperature, more than 1,000° C. may be conceived. Difference in shade is remarkable when the treating temperature is higher; difference in shade is difficult to see when the treating temperature becomes low and when the temperature is below the melting point of the filaments, different dyeability is completely not recognized. However, it should be noted that other elements are also important. Next problem is the treating time; the time is determined from a velocity at which the filaments to be treated pass through the heating zone and the passing length. Generally, when the heat treating time is too short, a sufficient effect of heat treatment cannot be obtained and it is not possible to achieve the objects of the present invention. The heat treating effect varies mainly by the heat treating temperature and time, and because the higher the temperature, the larger the heat treating effect, the time required for obtaining the predetermined heat treating effect may be short. Again, in the present invention, because the fibers of the polyester series are heat treated at a high temperature above the melting point of said fibers, when the heat treating time is too long, the fibers melt completely. Because of this, the longest heat treating time has a limit of itself, about which mention will be made in detail later. Finally, there is a problem of tensile strength of the filaments, which is preferably very weak. It is preferable to enable the filaments shrinking by heating to freely modify and this modification should not be restricted.

In the foregoing, the heat treating temperature is made  $T$  (° C.), the melting point of the fibers of the polyester series is made  $T_m$  (° C.) and the heat treating time is made  $t$  (sec.) and relation existing among them is determined.

It is perhaps impossible to theoretically analyze the present invention and the relationships involved are determined mainly based on the results obtained experimentally. In Table 1, results of practicing the process of the present invention are shown.

Upon carrying out a heat treatment, filaments to be treated were passed through a heating cylinder having an internal diameter of 8 mm. and a length of 30 cm. under tension imposed on said filaments of substantially zero.

In Table 1, in Nos. 1-14, the filaments treated were normally drawn and heat-set polyethylene terephthalate yarn (75 de./36 fil., inherent viscosity in o-chlorophenol at 35° C. of 0.62, draw ratio: 3.65, heat-set temperature: 170° C., shrinking in boiling water: 6%, degree of crystallinity: 47%), whereas in Nos. 15-19, the filaments treated were non-heat-set polyethylene terephthalate yarn (denier, inherent viscosity and draw ratio were same as in the cases of Nos. 1-14, shrinkage in boiling water: 12%, degree of crystallinity: 25%). In Table 1, (1) degree of shade was: (O)—remarkable, (Δ)—fairly good, and (X)—no difference in shade recognized.

(2) Degree of crystallinity was determined by an X-ray diffraction method, whereby the fiber axis was placed perpendicularly to an X-ray beam, an X-ray diffraction curve in a direction at a right angle with the fiber axis was measured and said degree could be simply determined by the following method. Namely, on both sides (a lower angle side and a higher angle side) of a peak of X-ray diffraction pattern in the vicinity of 17.5° C. in said X-ray diffraction curve, a line was depicted so as to contact an intensity of X-ray diffraction peak curve. From the highest point A of said peak of X-ray diffraction pattern, AC was depicted perpendicularly to said axis. AC showed an intensity of X-ray diffraction pattern at the point A, an intersecting point of AC with the previously depicted tangent was made B and degree of crystallinity was sought from  $AB/AC \times 100\%$ .

As will be apparent from Table 1, when the treating temperature was less than the melting point of the polyester +100° C., no difference in shade was obtained (Nos. 1, 2 and 3). Namely, even if the degree of crystallinity of the filaments was more than 40%, when the treating temperature was low, different dyeability could not be obtained.

By arrangement of the experimental results described above, Table 1 and other data, the primary variables

$T$ : heat treating temperature ° C.

$T_m$ : melting point of polyester ° C.

$t$ : treating time, sec.

were plotted on a sheet of logarithmic section paper to obtain empirical Formulas 1 and 2.

$$\log T - \log T_m = -0.688 - 0.588 \log t \quad (1)$$

and the treating temperature is necessarily not less than  $t$  defined by said Equation 1, and its upper limit is:

$$\log (T - T_m) = 1.576 - 1.085 \log t \quad (2)$$

Namely, the treating temperature is necessarily not more than  $t$  calculated by said equation 2. The reason  $T$ ,  $T_m$

TABLE 1

| Number  | Treating temp., ° C. | Forwarding velocity, m./min. | Withdrawing velocity, m./min. | Treating time, sec. | Crystallinity degree, percent | Degree of a shade of color | Shrinkage in boiling water | Remarks              |
|---------|----------------------|------------------------------|-------------------------------|---------------------|-------------------------------|----------------------------|----------------------------|----------------------|
| 1-----  | 250                  | 90                           | 75                            | 0.24                | 53                            | X                          | 0.5                        | Comparative example. |
| 2-----  | 300                  | 90                           | 75                            | 0.24                | 58                            | X                          | 0.4                        | Do.                  |
| 3-----  | 300                  | 174                          | 150                           | 0.12                | 53                            | X                          | 1.0                        | Do.                  |
| 4-----  | 360                  | 90                           | 75                            | 0.24                | 60                            | 0                          | 0.4                        | Do.                  |
| 5-----  | 360                  | 174                          | 150                           | 0.12                | 57                            | Δ                          | 0.8                        |                      |
| 6-----  | 360                  | 351                          | 300                           | 0.06                | 52                            | Δ                          | 2.0                        |                      |
| 7-----  | 400                  | 174                          | 150                           | 0.12                | 60                            | 0                          | 0.1                        |                      |
| 8-----  | 400                  | 351                          | 300                           | 0.06                | 55                            | 0                          | 1.0                        |                      |
| 9-----  | 400                  | 545                          | 450                           | 0.04                | 51                            | Δ                          | 2.8                        |                      |
| 10----- | 400                  | 608                          | 600                           | 0.03                | 48                            | X                          | 4.0                        |                      |
| 11----- | 500                  | 545                          | 450                           | 0.04                | 59                            | 0                          | 0.2                        |                      |
| 12----- | 500                  | 608                          | 600                           | 0.03                | 52                            | Δ                          | 1.0                        |                      |
| 13----- | 500                  | 962                          | 900                           | 0.02                | 40                            | X                          | 4.5                        |                      |
| 14----- | 1000                 | 825                          | 750                           | 0.24                | 55                            | 0                          | 0.5                        |                      |
| 15----- | 400                  | 284                          | 225                           | 0.08                | 56                            | 0                          | 0.5                        |                      |
| 16----- | 400                  | 545                          | 450                           | 0.04                | 42                            | 0                          | 2.7                        |                      |
| 17----- | 400                  | 608                          | 600                           | 0.03                | 35                            | X                          | 4.5                        | Do.                  |
| 18----- | 500                  | 608                          | 600                           | 0.03                | 45                            | 0                          | 1.0                        | Do.                  |
| 19----- | 500                  | 825                          | 750                           | 0.024               | 40                            | Δ                          | 1.0                        |                      |

and  $t$  are arranged as mentioned above is, even if it is called unconditionally high temperature heat treatment, its varying scope (combination of  $T$  with  $t$ ) is very broad, and there is a scope where different dyeability is not developed. For example, in said Equation 2, when  $t$  is made too large, it exceeds the upper limit, resulting in inconvenience. Namely, not only different dyeability is not developed, but also actually the filaments melt, inviting an entirely different result. On the contrary, as examples of making small  $t$ , in cases of Nos. 10, 13 and 18 the treating temperatures in said Equation 1 are within the range of the present invention, however, because the treating times are made less than  $t$ , it is understood that the objects are not achieved similarly.

When the description made so far is summarized, construction of the present invention is as follows.

(1) Fibers of the polyester series are made to pass through a high temperature atmosphere kept at a temperature higher than the melting point of said fibers.

(2) In the above case, fibers transfer under low tension (e.g. less than 0.03 g./de.)

(3) Relation among  $T$ ,  $T_m$  and  $t$  is according to the following empirical equation.

$$\log T - \log T_m = -0.688 - 0.588 \log t$$

(4) The final degree of crystallinity of the fibers after treatment is at least 40%.

In the present invention, upon carrying out a high temperature heat treatment, as the medium for heating the fibers, a gas is most suitable. Namely, a gas heated to the desired temperature is filled in the cylinder 2 shown in FIG. 3. For keeping the temperature constant a gas at a predetermined temperature may be supplied from an entrance 4 at one end and discharged from an exit 5 at the other end or the filaments may be passed through an electrically heated chamber.

As another kind of a heating apparatus, means of irradiating infrared ray to the filaments may be adopted. A heating apparatus of an optional type other than what is illustrated may be adopted. The heat treating temperature as herein referred to is a temperature of a heating medium in the vicinity of the surface of the fibers to be treated, which can be easily measured by, for instance, a thermocouple.

The fibers of the polyester series usable in the present invention are homopolyester or copolyester all or a main part of an acid component of which is terephthalic acid and all or a main part of a glycol component of which is ethylene glycol. A blend which is spun by the conventional process and further subjected to drawing or drawing followed by heat-set treatment is preferable, especially a multifilament yarn is most suitable.

When the filaments heat treated by the aforementioned process of the present invention and different dyeability state are observed, non-periodic as it is, a very clear shade of color is shown, the changing scope of the color tone is very short and it is possible to obtain a scope of several centimeters or even several millimeters. The fact that the filaments have such complicated different dyeability as mentioned above is very useful depending upon the desired use. Depending upon a dyeing method, for instance, in case of a print, it is possible to make almost invisible different dyeability and the dyed fibers may be offered for use wherein feel only is estimated.

Because the process of the present invention carries out a non-contact heat treatment, it is possible to treat the fibers continuously at a higher speed.

The fibers treated by the process of the present invention retain practical mechanical properties.

The fibers treated by the process of the present invention are imparted with different dyeability remarkable in distinction of a shade of color.

The fibers treated by the process of the present invention develop peculiar crimp, having special feel.

## EXAMPLE 1

Non-heat-set drawn polyethylene terephthalate filaments (75 de./36 fil., an inherent viscosity measured in o-chlorophenol at 35° C. of 0.61,  $\Delta n=0.141$ ) were passed through a cylindrical tube having a diameter of 1.9 cm. and a length of 30 cm. heated by electric heat to 550° C. and continuously heat treated in heated air at a withdrawing speed of 30 m./min. under tension of 0.0 g./de. (in the following example the same apparatus was used). The treated filaments obtained were finely crimped and by dyeing (dyeing for 30 minutes using Dispersal fast Scarlet B, dyeing in the following example was same as this), a shade of color at a cycle of about 2 cm. was brought about on said filaments. Filaments heat treated under conditions same as above except tension was changed to 0.04 g./de. exhibited no crimp, and when the filaments were dyed no periodic shade of color was recognized.

## EXAMPLE 2

A polyethylene terephthalate yarn having a Y-shaped cross section (50 de./48 fil.) was heat treated at 500° C. under tension of 0.01 g./de. and a withdrawing speed of 300 m./min. As a result of dyeing said yarn, a fine and remarkable shade of color having a cycle of about 5 mm. was brought about.

## EXAMPLE 3

Heat-set filaments of polyethylene terephthalate having copolymerized 5% by weight of polyethylene glycol (melting point: 258° C., 50 de./24 fil., inherent viscosity: 0.62,  $\Delta n=0.148$ , shrinkage in boiling water: 7.8%, shrinkage at dry heat of 150° C.: 9.5%) were heat treated at 500° C. under substantially no tension at a withdrawing speed from a heated zone of 300 m./min. As a result, filaments exhibiting a shade of color at a cycle of about 2 cm. were obtained. The shrinkage in boiling water of said treated fibers was 2.5% and shrinkage at dry heat of 150° C. was 3.0%.

## EXAMPLE 4

Polyethylene terephthalate filamentary yarn processed by a false twist method was heat treated at 550° C. under tension of substantially zero at a withdrawing speed of 300 m./min. As a result yarn having a difference in shade in a direction of length of about 15-20 cm. was obtained.

## EXAMPLE 5

Drawn heat-set polyethylene terephthalate filaments (75 de./36 fil., inherent viscosity in o-chlorophenol at 35° C. of 0.6,  $\Delta n=0.161$ ) were passed through a dry heated cylinder having an internal diameter of 8 mm. and a length of 30 cm. and continuously heat treated at 600° C. under tension of 0.005 g./de. at a withdrawing speed of 600 m./min. The so obtained filaments were finely crimped, and when dyed exhibited a remarkable shade of color at a cycle of about 2-3 cm.

The shrinkage in boiling water of said treated filaments was 0.4% and shrinkage at a dry heat of 150° C. was 0.5%.

What is claimed is:

1. A process for preparing a continuous multifilament yarn of a linear polyester, the filamentary yarn of which consists of deep-dyeing portion and pale-dyeing portion occurring alternatively along the axis of the said yarn, which process comprises passing a drawn polyester multifilament yarn through a high temperature stationary atmosphere maintained at a temperature ( $T$ ) at least 100° C. higher than the melting point ( $T_m$ ) of said polyester up to about 1000° C., for a period of time ( $t$ ) of 0.02 to 0.24 second, under a yarn tension of less than 0.03

gram per denier so that the final degree of crystallinity is at least 40%, the variables  $T$ ,  $T_m$  and  $t$ , satisfying the equations

$$\log T - \log T_m = -0.688 - 0.588 \log t \quad (1) \quad 5$$

$$\log (T - T_m) = 1.576 - 1.085 \log t \quad (2)$$

|           |         |              |           |
|-----------|---------|--------------|-----------|
| 3,156,752 | 11/1964 | Cope         | 264-342 R |
| 3,166,886 | 1/1965  | Kretsch      | 28-72     |
| 3,443,009 | 5/1969  | Chirgwin     | 28-61     |
| 3,022,564 | 2/1962  | Price        | 28-55.2   |
| 3,367,003 | 2/1968  | Scott        | 28-76 R   |
| 3,421,194 | 1/1969  | Breen et al. | 28-72.12  |
| 3,490,219 | 1/1970  | Ozawa et al. | 57-34     |

## References Cited

## UNITED STATES PATENTS

|           |         |                  |           |    |
|-----------|---------|------------------|-----------|----|
| 2,956,330 | 10/1960 | Potzl            | 264-342 R | 10 |
| 3,005,251 | 10/1961 | Hallden et al.   | 28-76     |    |
| 3,011,215 | 12/1961 | Alley            | 264-210 L |    |
| 3,069,836 | 12/1962 | Dahlstrom et al. | 264-342 R |    |

JAY H. WOO, Primary Examiner

U.S. CL. X.R.

8-14, 15, 149.3; 28-62; 264-235, 346